

## UNITED STATES PATENT OFFICE

2,227,311

## PROCESS FOR THE SYNTHESIS OF PLASTIC MATERIALS FROM UNSATURATED HYDROCARBON OILS AND SULPHUR

Herman B. Kipper, Accord, Mass.

No Drawing. Application May 6, 1938,  
Serial No. 206,352

10 Claims. (Cl. 260—67)

The novel descriptions, as believed by applicant, contained in the following application, represent a continuance of similar work covered by applications Serial Numbers 89,463; 100,818; 5 111,679; 148,960; 168,394; 179,270, and 187,897.

The specific findings covered more especially in this application pertain to the production of plastic materials produced from olefinic hydrocarbons, such as are given off as by-products in 10 the cracking of petroleum oils for fabrication of various commercial oils and more especially gasoline.

The reaction chamber used by applicant for carrying out his experimental investigations consists of a chrome-nickel-iron alloy tube about six feet long and one and one-half inches internal diameter and two and three-eighths inches external diameter. Heating of the tube was carried out by means of electric resistance furnaces.

20 Two "boats," or tubes, made of the same alloy, and slotted lengthwise with a half inch slot for filling, and each about thirty inches long, were used for introduction of the catalytic, or other reaction, materials into the reaction chamber before closing the same with steel plugs, lead gasketed.

As carried out in one of the experiments, into each boat was placed about twenty-five grams of sulphur, mixed with three grams of finely divided 30 antimony sulphide. There was then run into the reaction tube about two hundred and fifty grams of olefines, mostly butylenes. These were forced into the tube from another tubular container by means of nitrogen until some three hundred 35 pounds gauge pressure was registered. The tube was then closed and heated to about two hundred degrees centigrade during a period of twenty minutes and then gradually raised to a temperature of two hundred and fifty degrees over an 40 hour period. The heating was continued for about half an hour longer and the tube then allowed to cool. A viscous plastic-like material was thereby formed. About one hundred and fifty grams of product was obtained.

45 In other runs finely powdered iron and copper, litharge, magnesium oxide and "solid" cuprous acid phosphate, thiourea and other organic activators as piperidine and orthotoluidine were added to the sulphur. They did not appear to aid towards the formation of a better plastic. Shredded asbestos was also added to the sulphur to render it more "open" for reactioning, but the character of the finished plastics remained nevertheless fairly alike. In other words, a viscous 50 tough product was formed rather than a hard

plastic. This product, applicant found, could be considerably hardened and a truer plastic produced by treatment with an aldehyde, as formaldehyde, acetaldehyde, croton aldehyde, benzaldehyde and furfural. The latter gave the best 5 product. The viscous product as produced in the reaction chamber was simply thoroughly mixed with the aldehyde and a condensation agent. Barium oxide acted especially advantageously for this purpose. Sodium hydroxide, anhydrous ammonia, aluminum chloride, sodium sulphide and sodium thiosulphate were also tried and established reaction between the synthesized product and the aldehyde. From five to twenty percent of the latter were used, on basis of synthesized 10 product, and five to fifteen percent of the condensation reagents. Heating of the reaction mass was conducted at one hundred to one hundred and fifty degrees centigrade under high 15 pressure.

20 In my next set of experiments the rear boat of the reaction tube initially was more or less similarly filled with sulphur, comingled with the various materials such as already noted. The front boat, however, was filled with a mixture of copper 25 and iron oxides carried by shredded asbestos. The basic differences in experimentation were due to the use of oxygen with the olefinic gases so as to produce oxidation of the latter. Also oils produced according to my application Serial 30 Number 187,897 from olefinic gases were oxidized concurrently with the reaction used for plastic formation, or they were previously oxidized and then utilized for the reactions in question.

Methods employed for carrying out the latter 35 reaction, that is, those conducted under an oxidizing atmosphere, were as follows:

Two hundred and fifty grams of olefines, mostly butylenes, were run into a steel cylinder of about forty-five liters capacity and the latter was then 40 filled to two hundred and fifty pounds gauge pressure with a ninety-five percent nitrogen, five percent oxygen mixture.

The gas mixture, containing the olefines, was then circulated through the reaction tube, heated 45 to two hundred and twenty-five degrees centigrade for about an hour at the rate of about one liter per minute. This method proved only semi-satisfactory, as the vapor tension of the butylenes proved to be too low under the operating conditions to give the gas mixture sought. In our next experiment along these lines the olefines were pumped separately through the reaction chamber and the nitrogen-oxygen mixture was also circulated separately but simultaneously. In a 50 55

third experiment an oil produced from olefines, according to my application Serial Number 187,897 was pumped through the reaction chamber at the rate of about two hundred and fifty 5 cubic centimeters per hour and the oxidizing gas was circulated as described in the last experiment. In another experiment the above oil was oxidized with five percent fuming nitric acid after addition of about two percent aluminum chloride 10 to the oil and heating of the same to between fifty and one hundred degrees centigrade. Other hydrolyzing metal chlorides, as those of iron, copper, tin and antimony, were also used for this purpose. The oxidation was carried out under powerful 15 stirring. The oxidized oil was then mixed with about forty percent of sulphur, two percent antimony sulphide, ten percent furfural and three percent barium oxide and heated to one hundred and fifty degrees in a closed tube. By all of these 20 latter four methods, hard plastics were produced. Some of the yields secured were poor, but it is applicant's belief that such poor yields were due rather to experimental difficulties than to lack of completion of reaction. In the last mentioned 25 experiment all raw materials utilized were incorporated into the finished plastic.

These oxidized oils, I am now also investigating in paints or "drying oils." With a small percentage of rubber, about one percent, incorporated with them, very excellent drying oils and of commercial viscosities are secured. Rubber is very soluble in the oil. Also polymerizations of the oils are being conducted with sodium and other condensation agents. I have secured products resembling rubber through such application 30 for a period of six weeks. Furthermore, I have carried out oxidations of ordinary fuel and other heavy petroleum oils with aluminum chloride and nitric acid of various concentrations and secured 35 thereby most excellent drying oils, especially when used in the presence of ammonium chloride as a polymerizing or oxidizing agent in the paint films.

It is my belief that I have outlined my methods 40 of production sufficiently in detail to permit of clear-cut, easy reproduction and thus shall give but a further example or two of operations, as details of all the "runs" made would hardly add anything further novel or of value to the art.

50 One of the boats of my reaction tube was filled with twenty-five grams of sulphur, two grams of antimony sulphide, three grams of barium oxide and twenty-five grams of croton aldehyde and the other boat similarly filled with the exception 55 that the barium oxide was replaced by "solid" cuprous acid phosphate. A few grams of shredded asbestos was also comingled with the reaction masses of sulphur, etc. The reaction tube was closed and two hundred and fifty grams of olefines, mostly butylenes, were forced into the tube 60 by nitrogen gas until the reaction tube registered three hundred pounds gauge pressure. The tube was then raised rapidly to two hundred degrees and maintained at the latter temperature for 65 three hours. The reaction tube was opened subsequently to cooling. Hard, excellent plastics were secured. About two hundred and fifty grams of plastic material were obtained. A plastic made 70 according to the above method in which heating, after the reaction temperature had been reached, was continued for only an hour, was tough and viscous in character. Thus it will be noted that "hardness" securable in the finished plastic is 75 dependent upon the period of heating or of

reaction and that this specific quality is enhanced as the said period is lengthened.

With furfural I used only a hundred and fifty degree reaction temperature. The same temperature was employed when using benzaldehyde and 5 salicylaldehyde.

In my final work the oils, treated with hydrolyzing metal chlorides, as aluminum chloride, cupric chloride, antimony chloride or ferric chloride and nitric acid, were further polymerized by allowing to stand for several weeks at room temperatures, or heated to a temperature of fifty to sixty degrees centigrade, in the presence of a small percentage of aluminum chloride. The oils were thereby further polymerized to give viscous 15 elastic-like masses. Treatment with sulphur, or sulphur and antimony chloride, was then conducted at one hundred and fifty to two hundred degrees centigrade in my reaction tube, either at atmospheric pressure or under superatmospheric 20 pressures exerted by an inert gas, as nitrogen. From twenty-five to fifty percent of sulphur was used and small percentages of antimony sulphide. With ten to fifteen percent of sulphur, tough, elastic materials resembling vulcanized 25 rubber were secured. Small percentages of so-called rubber accelerators were likewise employed, especially those used with synthetic rubbers, as piperidine, thiourea and orthotoluidine. Also to destroy any aluminum chloride that might remain 30 in the tough viscous mass used for plastic formation, a small percentage of sodium sulphide was incorporated with and thoroughly worked into the said mass. Also aldehydes were used in the reaction, ten to twenty percent. Croton alde- 35 hyde and furfural hardened the plastics formed, but in all cases where over thirty percent of sulphur was used relatively hard, excellent plastics were produced. Rubber, up to ten percent, was also added to the oils or viscous masses before 40 plastic formation. As has been noted, rubber is very soluble in the oils and the quality of the plastic formed through its incorporation appeared 45 possibly better.

I also experimented with adding urea, thiourea 45 and phenol to the sulphur mass. The aldehydes were then used in excess proportions to those required for plastic formation from the chemicals just mentioned. Thus, plastics well known to the art were produced simultaneously and as a part 50 of, or comingled with, my novel plastic materials. In this manner, plastics having a very wide range of properties can be fabricated.

As to be probably expected, the viscous elastic-like masses produced by treatment of the condensed olefines with aluminum chloride and nitric acid, when reacted with sulphurchlorides, either the mono- or di-chloride, give first tough pliable 55 elastic bodies and as the percentage of the sulphurchloride is increased, hard plastic materials 60 are formed. The percentage of the sulphurchloride used was made as high as one hundred percent before the plastic showed any noticeable decomposition, that is, with the formation of free carbon.

These plastics show thermoplastic qualities, softening between one hundred and fifty and two hundred degrees centigrade, at which temperatures they can be readily pressure molded.

Applicant believes that the examples cited illustrate basically his novel processing for plastic 70 fabrications. Combinations of raw material specifications, operating conditions could, of course, be multiplied ad infinitum without actually digressing from his basically novel findings. 75

I claim:

1. In a process for the production of plastic materials the step of reacting olefines, organic aldehydes and sulphur at superatmospheric pressures and temperatures.
  2. In a process for the production of plastic materials the step of reacting olefines, organic aldehydes, sulphur and antimony sulphide at superatmospheric pressures and temperatures.
  3. In a process for the production of plastic materials the step of reacting olefines, organic aldehydes, sulphur and antimony sulphide at superatmospheric temperatures and pressures, the latter partially maintained by means of an inert gas.
  4. In a process for the production of plastic materials the step of reacting olefines, sulphur and unsaturated hydrocarbon oils, previously treated with hydrolyzing metal chlorides and nitric acid, at superatmospheric temperatures and pressures.
  5. In a process for the production of plastic materials the step of reacting olefines, sulphur, aldehydes and unsaturated hydrocarbon oils, previously treated with hydrolyzing metal chlorides and nitric acid, at superatmospheric temperatures and pressures.
  6. In a process for the production of plastic materials the step of reacting olefines, sulphur, antimony sulphide, aldehydes and unsaturated hydrocarbon oils, previously treated with hydrolyzing metal chlorides and nitric acid, at superatmospheric temperatures and pressures.
  7. In a process for the production of plastic
- materials the step of reacting olefines, condensed at superatmospheric pressures and temperatures to oils and treated with hydrolyzing metal chlorides and nitric acid subsequently to condensation, with sulphur at superatmospheric temperatures.
8. In a process for the production of plastic materials the step of reacting olefines, condensed at superatmospheric pressures and temperatures to oils and treated with hydrolyzing metal chlorides and nitric acid subsequently to condensation, with sulphur at atmospheric temperatures and pressures, the latter partially maintained by means of an inert gas.
9. In a process for the production of plastic materials the step of reacting olefines, condensed at superatmospheric pressures and temperatures to oils and treated with hydrolyzing metal chlorides and nitric acid subsequently to condensation, with sulphur, antimony sulphide, litharge, piperidine and thiourea at superatmospheric temperatures and pressures, the latter partially maintained by means of an inert gas.
10. In a process for the production of plastic materials the step of reacting butylenes, condensed at superatmospheric pressures and temperatures to oils and treated with aluminum chloride and nitric acid subsequently to condensation, with sulphur, antimony sulphide, litharge, piperidine and thiourea at two hundred degrees centigrade and two hundred pounds pressure, said pressure maintained by means of nitrogen.

HERMAN B. KIPPER.